# EUROPEAN PATENT SPECIFICATION

(11) **EP 2 210 677 B1**
(45) Date of publication and mention of the grant of the patent: **28.03.2012**
(21) Application number: 10151246.5
(22) Date of filing: 20.01.2010
(51) Int. Cl.: B08B 3/12, H01L 21/02, C11D 7/06, C11D 7/10, C11D 7/14

(54) **Cleaning solution and cleaning method for an electrical conductor**
Reinigungslösung und Reinigungsverfahren für elektrische Leiter
Solution de nettoyage et procédé de nettoyage de conducteur électrique

(30) Priority: 22.01.2009 US 357610; 29.10.2009 US 608079
(43) Date of publication of application: 28.07.2010
(73) Proprietor: Electric Power Research Institute, Inc., Charlotte, NC 28262 (US)
(72) Inventor: Phillips, Andrew J., Charlotte, NC 28262 (US); Stewart, Andrew H., Fort Collins, CO 80526 (US); Ningileri, Shridas, Lexington, KY 40513 (US); Hurst, Neil J., Fort Collins, CO 80525 (US); Bush, J. Finely, Leechburg, PA 15656 (US); Xia, Sike, Pearland, TX 77584 (US); Xiao, Chenghe, Lexington, KY 40513 (US); Liu, Yansheng, Lexington, KY 40509 (US)
(74) Representative: Moy, David

(56) References cited:
- EP-A1- 1 160 312
- EP-A1- 1 338 645
- WO-A1-01/20653
- WO-A2-2006/110645
- GB-A- 2 449 759
- JP-A- 2007 194 615
- US-A1- 2002 139 393
- US-A1- 2004 118 432
- US-A1- 2005 227 363
- US-A1- 2007 161 529

## Description

### BACKGROUND OF THE INVENTION

The present invention relates generally to a conductor cleaning system, and more particularly to a system for cleaning aluminum strands of all aluminum and steel reinforced electrical conductors, such as ACSS, ACSR, ACAR, and AAA.

In current power transmission systems, failures can pose a significant risk to the reliability of the system. There are several factors that contribute to these failures - one such factor is the failure of compression connectors.

Current data suggests that a primary root cause for failures in compression connectors is improper installation. Examples of improper installation include lack of compound, alignment, wrong die, and poor cleaning of the aluminum strands of the conductor prior to installation of compression connectors. Research indicates that corrosion products and other contaminants (resulting from years of exposure to the environment) left on the conductors during splice assembly can raise the resistance of the splice-conductor joint (this is also true of new conductors which have oxidation and contaminants thereon). Cyclical variations of load current feeding through the increased resistance of the splice-conductor joint causes thermal expansion/contraction that eventually reduces the grip of the splice to a point where it can no longer hold the conductor.

Currently, compression connector installers clean the aluminum strands with a wire brush, which results in ineffective cleaning of the strands, leaving corrosion products and other contaminants behind. Further, the installer cannot clean internal strands using the wire brush unless the installer takes the time to unstrand the conductor. Unfortunately, unstranding is impractical in most field conditions and can increase the risk of damage to the individual strands.

EP 1160312 A1 (to Yasuo Sadoyama) discloses a detergent composition which contains sodium (III) phosphate, sodium metasilicate, sodium sulfate, sodium tripolyphosphate, sodium chloride, sodium carbonate, and at least one or more of compounds selected from potassium chloride, trisodium citrate and sodium hydroxide. GB 2449759 A (to General Electric Company) discloses a method for cleaning a generator coil using an ultrasonic cleaning system including an aqueous solution being, for example, a caustic solution including sodium hydroxide. US 2002/139393 A1 (to Annette Crevasse et al) discloses a wafer cleaning apparatus including cleaning brushes mounted within a brush box and a sensor associated with at least one of the cleaning brushes and configured to detect a degree of wetness of the at least one of the cleaning brushes. WO 01/20653 A1 (to Koninklijke Philips Electronics N.V.) discloses an arrangement or method for detecting the end of life of an aqueous bath utilized in semiconductor processing, the bath containing water, an amount of hydrogen peroxide and an amount of a predetermined chemical species. US 2005/227363 A1 (to Hwang Dong-Won et al) discloses a method for monitoring metal contamination of a rinsing solution, the method comprising providing a sample of the rinsing solution, mixing the simple of the rinsing solution with a monitoring reagent to provide a monitoring mixture, and measuring a property of the monitoring mixture that is dependent on a concentration of a metal in the rinsing solution.

JP 2007 194 615 A discloses a cleaning composition for a semiconductor manufacture device that is based on phosphoric acid and/or phospate and further comprises a fluorine compound selected from among sodium fluoride, potassium fluoride, lithium fluoride and ammonium fluoride.

Accordingly, there is a need for a conductor cleaning system that can effectively clean both outer and inner strands of a conductor without the need to unstrand the conductor.

### BRIEF SUMMARY OF THE INVENTION

These and other shortcomings of the prior art are addressed by the present invention, which provides a conductor cleaning system capable of cleaning external and internal strands of a conductor without unstranding the conductor.

According to one aspect of the present invention, a conductor cleaning system includes a container adapted to receive a portion of a conductor to be cleaned, a housing adapted to receive and support the container, and a cleansing solution contained in the container for cleaning the portion of the conductor. The cleaning solution is adapted to clean the conductor without reacting with or damaging the conductor.

According to another aspect of the present invention, a cleaning solution adapted to clean electrical conductors, comprising: a caustic composition including a hydroxide cleaning agent, and wherein the caustic composition further includes NaF.

Suitably, the hydroxide cleaning agent is sodium hydroxide (NaOH).

Suitably, the caustic composition further includes NaF to enhance the solubility of aluminum oxides and reduce the time needed to complete a cleaning of an electrical conductor.

According to another aspect of the present invention, a cleaning solution adapted to clean electrical conductors without damaging galvanization coatings or degrading aluminum contained in the coatings or conductor has a composition, by approximate weight percent, of 0.985 to 8.97 NaOH, 0.49 to 1.45 NaF, and 89.7 to 98.5 H₂O

According to another aspect of the present invention, a cleaning solution adapted to clean electrical conductors without damaging galvanization coatings or degrading aluminum contained in the coatings or conductor has a composition, by weight percent, of 0.985 to 8.97 NaOH, 0.49 to 1.45 NaF, and 89.7 to 98.5 H₂O

It will be appreciated that simple mathematics dictates that the sum of the percentages of the components of any defined cleaning solution cannot exceed 100%.

By "approximate weight percent", it is meant that one should construe the ranges of values as would be understood by a person skilled in the art.

According to another aspect of the present invention, a method of cleaning an electrical conductor according to claim 11 includes providing a conductor cleaning system having a container and an agitator. The method further includes providing a cleaning solution for cleaning of the electrical conductor, introducing the cleaning solution into the container, positioning an electrical conductor in the cleaning solution disposed in the container, and activating the agitator, thereby agitating the cleaning solution and enhancing its ability to clean the electrical conductor.

Suitably, the method further comprises the step of checking the pH of the cleaning solution before and after cleaning the electrical conductor.

Suitably, the method further comprises replacing the cleaning solution with a new cleaning solution when the pH of the cleaning solution indicates that the cleaning solution is ineffective in cleaning the electrical conductor.

### BRIEF DESCRIPTION OF THE DRAWINGS

The subject matter that is regarded as the invention may be best understood by reference to the following description taken in conjunction with the accompanying drawing figures in which:

Figure 1 is a perspective view of a conductor cleaning system according to an embodiment of the invention;

Figure 2 shows a vibrator housing of the conductor cleaning system of Figure 1;

Figure 3 shows an eccentric weight for use in a vibrator of the conductor cleaning system of Figure 1;

Figure 4 shows a battery and receptacle for the conductor cleaning system of Figure 1;

Figure 5 shows a control panel for the conductor cleaning system of Figure 1;

Figure 6 shows the conductor cleaning system of Figure 1 being carried;

Figure 7 shows the conductor cleaning system of Figure 1 in use;

Figures 8 -10 show the conductor cleaning system of Figure 1 supported in an upright position by supports;

Figure 11 shows the conductor cleaning system of Figure 1 fitted with bipods;

Figure 12 shows a tri-pod for supporting the conductor cleaning system of Figure 1;

Figure 13 is a perspective view of a conductor cleaning system according to an embodiment of the invention; and

Figure 14 is a graph showing pH v. cleaning sequence.

### DETAILED DESCRIPTION OF THE INVENTION

Referring to the drawings, an exemplary conductor cleaning system according to the present invention is illustrated in Figure 1 and shown generally at reference numeral 10. The system 10 includes a container, such as tube 11 operably connected to an agitator, such as vibrator 12, Figure 2, contained in a vibrator housing 13, and a control panel 14 for controlling the system 10. The container 11 may be disposable or permanently attached to the system 10.

The vibrator housing 13 is adapted to receive and support the container 11, and includes an attachment rail 16 to allow the system 10 to be attached to a support for easy operation or to allow a user to easily carry the system 10. Other attachments such as a hook-type attachment may also be used to attach the system 10 to a bucket of a bucket truck or other suitable support. A standing base 17 is disposed at one end of the housing 13 to allow the system 10 to be positioned in a stand-up position such that the tube 11 is in a vertical position. The base 17 may be adapted to accept supports to further stabilize the system 10 in the vertical position, as shown in Figures 8-10. Guide straps 18 and 19 are attached to opposing ends 20 and 21 of the housing 13 to provide guides and supports for the tube 11, and a retaining strap 22 is positioned between the guide straps 18 and 19 to lock the tube 11 into position. A support 23 is also positioned on a bottom of the housing 13 to further position and lock the tube 11 into position. As shown, the support 23 is V-shaped; however, any suitable geometry may be used to position and lock the tube 11 in position.

As shown in Figure 2, the vibrator housing 13 includes a control system 30 having an electric motor 31, a timer circuit 32, a voltage regulator 33, and the vibrator 12. The vibrator 12 includes an eccentric weight 15, like that shown in Figure 3, to emit vibrations into the tube 11, thereby agitating a cleaning solution contained therein. While a vibrator is being described herein, it should be appreciated that other types of agitators may be used, for example, ultrasonic, bubbling air, and stirring. Together, the motor 31 and vibrator 12 cause the system 10 to vibrate at a specified rate by spinning the eccentric weight 15 at a desired speed. It should be appreciated that the speed of the motor 31 and size of the eccentric weight 15 may be changed to optimize the conductor cleaning efficiency. It should be appreciated that other forms of vibrators/agitators may be used, such as ultrasonic.

Referring to Figure 4, the system 10 is powered by a battery 36. The battery 36 is contained in a battery receptacle 37 of the base 17. The battery 36 may be replaceable or rechargeable and allows the system 10 to be portable for conductor cleaning both at ground level and at elevated levels.

As illustrated in Figure 5, the control panel 14 is electrically connected to the control system 30 and includes a power switch 38, a timer 39, a start button 40, and a buzzer 41. The power switch 38 turns the system 10 on to a ready state so that the system 10 is ready to clean a conductor. The timer 39 allows a user to choose how long the cleaning process is going to last. The amount of time chosen is dependent on the level of contaminants and corrosion products on the surface of the conductor, temperatures, and other factors. The start button 40 turns the cleaning process on when depressed, and the buzzer 41 lets a user know when the cleaning process has ended.

The cleaning solution is contained in the tube 11 to allow an end of a conductor to be cleaned properly while reducing spills and splashes. The cleaning solution is designed and optimized to permit cleaning of aluminum strands of conductors without unstranding the conductor. Namely, the cleaning solution is designed to permit internal and external cleaning of aluminum strands of the conductor without reacting and damaging the galvanization of galvanized steel strands; to not react with or degrade aluminum strands after the cleaning process is complete; to clean over a wide range of temperatures; to not react with inhibitor compounds used in compression connector installation; and to be environmentally acceptable.

The cleaning solution uses a caustic solution of sodium hydroxide (NaOH) as a cleaning agent due to the tri-hydrated oxide of aluminum found in corrosion products being soluble in this type of solution. It should be appreciated that other suitable caustic hydroxides may be used. The caustic level of the solution is equal to, or less than, that of standard household cleaners. A low concentration of sodium fluoride (NaF) enhances the solubility of the aluminum oxides and reduces the time needed to complete the cleaning. The predominant reactions occurring during cleaning are as follows:

Al₂O₃ + 2NaOH ⇔ 2NaAlO₂ +H₂O

2Al + 2NaOH +2H₂O → 2NaAlO₃ + 3H₂.

The reaction products are essentially stable and do not react with Al and the corrosion layer Al₂O₃. Only NaOH chemically attacks both Al and Al₂O₃. Examples of cleaning solutions are shown in the Table below.

| Solution | | Caustic Level |
|---|---|---|
| No. | Composition | |
| 1 | NaOH + H₂O | High |
| 2 | NaOH + NaPO₄•12H₂O + NaF + H₂O | Medium |
| 3 | NaOH + NaPO₄•12H₂O + NaF + H₂O | Medium-Low |
| 4 | NaOH + NaF+H₂O | Low |

In testing, all of the above solutions provided good to excellent cleaning results. For example, in one test, a cleaning solution having a low level of causticity and relatively simple composition was chosen. The cleaning solution had the following concentrations:
Sodium Hydroxide (NaOH) = 20g (approx. weight percent = 1.93)
Sodium Fluoride (NaF) = 15g (approx. weight percent = 1.45)
Water (H₂O) = 1 L. (approx. weight percent = 96.62)
It should be appreciated that other concentrations could be used depending on the application. For example, it was found that solutions having approximate weight percent ranges of 0.985 to 8.97 NaOH, 0.49 to 1.45 NaF, and 89.7 to 98.5 H₂O were acceptable. The chemicals were mixed in the water until completely dissolved. It was determined that the level of cleaning and the time to achieve that level were dependent on the solution temperature and the amount of agitation provided to the solution by the vibrator 12. This can be seen in the table below.

| Temperature (C) | Cleaning Effectiveness Rated 0 to 5 with 5 Being the Best | | | | | |
|---|---|---|---|---|---|---|
| | With Agitation | | | Without Agitation | | |
| | 1 Min | 2.5 Min | 5 Min | 1 Min | 2.5 Min | 5 Min |
| 0 | 3 | 4 | 4 | 1 | 1 | 2 |
| 25 | 4 | 5 | 5 | 2 | 3 | 4 |
| 50 | 5 | 5 | 5 | 5 | 5 | 5 |
| 70 | 5 | 5 | 5 | 5 | 5 | 5 |

It should be appreciated that other forms of agitation may be used, such as ultrasonic, bubbling air, stirring, etc.

When using a cleaning solution with ACSS and other conductors having aluminum incorporated into the steel core's zinc coating, care must be taken to prevent damaging the aluminum in the Al-Zn coating that protects the steel strands of the electrical conductor. The Al-Zn coating protects the steel strands from corrosion and degradation of the coating would be detrimental to the life of the electrical conductor. As a result, it was determined that the use of an inhibitor in the cleaning solution would be beneficial.

It was found that an inhibitor such as sodium silicate (Na₂O(SiO₂)ₓ(H₂O)ₓ) protected the Al-Zn coating while allowing the cleaning solution to adequately clean the electrical conductor. It was further found that a approximate weight percent range of 0.15 to 1.42 of sodium silicate was acceptable. When mixing the sodium silicate with the cleaning solution it was found that a solution, by approximate weight percent, suitably by weight percent, of (0.15 to 1.42) Na₂O(SiO₂)ₓ(H2O)ₓ + (1.90 to 1.93) NaOH + (1.43 to 1.45) NaF + (95.24 to 96.47) H₂O adequately cleaned the electrical conductors and protected the Al-Zn coating.

In addition to preventing damage to the Al in the Al-Zn coating, the pH is a concern due to EPA regulations for handling chemical solutions. Thus, it is beneficial to maintain the cleaning solution below a pH of 12.5. It was found, that various chemicals could be used to lower the pH of the solution. For example, it was found that a CaCl₂ solution could lower the pH from 13.0 to 12.4. However, the CaCl₂ solution tends to leave a residue.

It was further found that the use of ascorbic acid provided many benefits that the other chemicals did not. For example, the ascorbic acid was beneficial for both lowering the pH and for protecting the Al-Zn coating. A suitable and acceptable range, by approximate weight percent, suitably by weight percent, of ascorbic acid was found to be 0.193 to 3.54. This results in a cleaning solution having a composition, by approximate weight percent, of (0.193 to 3.54) ascorbic acid + (1.87 to 1.93) NaOH + (1.40 to 1.45) NaF + (93.28 to 96.43) H₂O.

In addition to lowering the pH and protecting the Al-Zn coating, when using the ascorbic acid, it was unexpectedly found that after a certain number of cleanings the pH of the cleaning solution dramatically fell off (See Figure 14), thereby indicating the need to change the cleaning solution before cleaning any more conductors. This is extremely beneficial because by simply monitoring the pH of the solution, a user knows exactly when to change out the solution for optimum cleaning.

As can be seen from Figure 14, a cleaning solution without ascorbic acid maintains a fairly constant pH across the cleaning sequences. On the other hand, the ascorbic modified cleaning solution steadily decreases in pH until the cleaning solution becomes ineffective (indicated by the sudden drop off in pH). As such, a user cleaning multiple conductors can monitor the pH of the ascorbic modified solution and easily determine a normal range of drop in pH either visually by graphing pH measurements prior to and after each cleaning, as done in Figure 14, or by calculating the drop in pH for each cleaning using the pH measurements and then determining a normal range of drop in pH. If during a cleaning, a drop in pH of the cleaning solution exceeds the normal range, then the user knows to dispose of the spent cleaning solution and replace it with new cleaning solution.

In use, the tube 11 is inserted through the guide straps 18 and 19 of the vibrator housing 13 and secured in position by the retaining strap 22 and support 23. As discussed, the tube 11 may be disposable or permanently attached to the system 10. In the case of a disposable tube, the tube 11 may be pre-filled with the cleaning solution and a plug 42 would be inserted into an end of the tube 11 to prevent spilling of the solution. The tube would then be attached to the system 10 and carried, as shown in Figure 6, to the conductor cleaning site. After use, the tube 11 would be removed from the system 10 and the tube and cleaning solution would be properly disposed of.

In the case of a permanent tube, the tube 11 would be attached to the system 10 and carried to the conductor cleaning site. The cleaning solution could be poured into the tube 11 and sealed therein by the plug 42 prior to delivery to the cleaning site, could be delivered to the site in another container and then poured into the tube at the site, or could be in powder form which would be mixed with water at the site.

Referring to Figure 7, once at the conductor cleaning site, a conductor 43 is inserted into the tube 11 so that the cleaning solution contained therein may clean the strands of the conductor 43. A baffle 44 may be inserted into the end of the tube 11 to prevent splashing during the cleaning process. With the conductor 43 positioned in the cleaning solution, the power switch 38 is moved to the on position and the timer 39 is moved to a desired time limit. The duration of vibration is determined by the user depending on the present temperature and the amount of deposits on the conductor surfaces. The start button 40 is then depressed and the motor rotates the eccentric weight 15 of the vibrator 12, thereby causing vibrations to agitate the cleaning solution to ensure that internal and external strands of the conductor are cleaned.

As discussed, during the cleaning cycle of the conductor, the system 10 may be supported in various ways to relieve the burden, on the user, of supporting the system 10. For example, if the system is to be supported in a vertical position, supports may be attached to the base 17, Figures 8-10. As shown in Figure 8, legs 46 are directly attached to the base 17. Legs 46 may be secured to the base 17 using fasteners. As illustrated in Figure 9, removable legs 47 are secured to the base 17 by pins 48. This allows the legs 47 to be removed when supporting the system 10 in a vertical position is not necessary. As shown in Figure 10, foldable legs 50 are secured to the base 17 by supports 49 which allow the legs 50 to pivot between a use position and a non-use position about pin 51.

Other support methods may also be employed. For example, in Figure 11, a bi-pod having legs 53 and 54 may be attached to strap 18. The legs 53 and 54 may be moved between a use position and a non-use position to allow the system 10 to be supported in a non-vertical position. As shown in Figure 12, a tri-pod 60 may also be used to support the system 10. As shown, the tri-pod 60 includes adjustable legs 61, 62, and 63 to allow for adjustment on uneven surfaces. The system 10 is then hung from the tri-pod 60 using the attachment rail 16.

Referring to Figure 13, a conductor cleaning system 110 is shown. Like system 10, system 110 includes a container 111 operably connected to a vibrator contained in a vibrator housing 113, a control panel 114, an attachment rail 116, a base 117, and retaining straps 118, 119, and 122. Unlike system 10, the container 111 of system 110 is a trough-like container to allow cleaning of a conductor 143 at a point intermediary of opposing ends of the conductor 143 without cutting. This allows the conductor 143 to be cleaned at locations where compression fittings, such as repair sleeves and T-connections, are being installed along the conductor 143.

In use, the container 111 is positioned at a point along the conductor 143 where cleaning is desired and moved into engagement with the conductor 143. Seals 160 and 161 permit the conductor 143 to be pressed into the container 111 until the conductor 143 is immersed in the cleaning solution. The seals 160 and 161 prevent the cleaning solution from leaking between the container 111 and the conductor 143.

The foregoing has described a conductor cleaning system. While specific embodiments of the present invention have been described, it will be apparent to those skilled in the art that various modifications thereto can be made without departing from the spirit and scope of the invention. Accordingly, the foregoing description of the preferred embodiment of the invention and the best mode for practicing the invention are provided for the purpose of illustration only and not for the purpose of limitation.

Although a few preferred embodiments have been shown and described, it will be appreciated by those skilled in the art that various changes and modifications might be made without departing from the scope of the invention, as defined in the appended claims.

## Claims

1. A cleaning solution adapted to clean electrical conductors, comprising: a caustic composition including a hydroxide cleaning agent, and wherein the caustic composition further includes NaF.

2. The cleaning solution according to claim 1, wherein the caustic composition, by approximate weight percent, comprises 0.985 to 8.97 NaOH.

3. The cleaning solution according to claim 1, wherein the caustic composition, by approximate weight percent, comprises 0.49 to 1.45 NaF.

4. A cleaning solution according to claim 1, having a composition comprising, by approximate weight percent, 0.985 to 8.97 NaOH, 0.49 to 1.45 NaF, and 89.7 to 98.5 H₂O.

5. The cleaning solution according to any preceding claim, further including, by approximate weight percent, 0.15 to 1.42 Na₂O(SiO₂)ₓ(H2O)ₓ.

6. The cleaning solution according to claim 5, wherein the cleaning solution comprises, by approximate weight percent, 0.15 to 1.42 Na₂O(SiO₂)ₓ(H2O)ₓ, 1.90 to 1.93 NaOH, 1.43 to 1.45 NaF, 95.24 to 96.47 H₂O.

7. The cleaning solution according to any of claim 1 to 4, further including, by approximate weight percent, 0.193 to 3.54 ascorbic acid.

8. The cleaning solution according to claim 7, wherein the cleaning solution comprises, by approximate weight percent, 0.193 to 3.54 ascorbic acid, 1.87 to 1.93 NaOH, 1.40 to 1.45 NaF, 93.28 to 96.43 H₂O.

9. The cleaning solution according to any of claims 4 to 8, further including an inhibitor to prevent degradation of aluminum in the galvanization coatings or the conductor.

10. The cleaning solution according to any of claims 4 to 9, further including an acid to control pH of the cleaning solution such that the pH is maintained below 12.5.

11. A method of cleaning an electrical conductor, comprising:
(a) providing a conductor cleaning system heaving:
(i) a container; and
(ii) an agitator;
(b) providing a cleaning solution as claimed in any one of claims 1 to 10 for cleaning of the electrical conductor;
(c) introducing the cleaning solution into the container;
(d) positioning an electrical conductor in the cleaning solution disposed in the container; and
(e) activating the agitator, thereby agitating the cleaning solution and enhancing its ability to clean the electrical conductor.

12. The method according to claim 11, wherein the cleaning solution comprises, by approximate weight percent, 0.15 to 1.42 Na₂O(SiO₂)ₓ(H2O)ₓ, 1.90 to 1.93 NaOH, 1.43 to 1.45 NaF, 95.24 to 96.47 H₂O.

13. The method according to claim 11, wherein the cleaning solution comprises, by approximate weight percent, 0.193 to 3.54 ascorbic acid, 1.87 to 1.93 NaOH, 1.40 to 1.45 NaF, 93.28 to 96.43 H₂O.

14. A method of determining when to replace a cleaning solution as claimed in any one of claims 1 to 10 in a conductor cleaning system with a new cleaning solution, comprising:
(a) measuring a pH of the cleaning solution prior to and after each cleaning of multiple electrical conductors;
(b) calculating a drop in pH of the cleaning solution for each cleaning using the pH measurements taken prior to and after each cleaning of the electrical conductors;
(c) determining a range of drop in pH using the calculated drops in pH for each cleaning; and
(d) replacing the cleaning solution with the new cleaning solution when a calculated drop in pH exceeds the determined range of drop in pH.

15. Use of a cleaning solution as claimed in any of claims 1 to 10 to clean electrical conductors.

## Patentansprüche

1. Reinigungslösung zum Reinigen von elektrischen Leitern, umfassend eine Laugenzusammensetzung, die ein Hydroxid-Reinigungsmittel enthält, wobei die Laugenzusammensetzung ferner NaF enthält.

2. Reinigungslösung nach Anspruch 1, wobei die Laugenzusammensetzung ungefähr 0,985 bis 8,97 Gew.-% NaOH umfasst.

3. Reinigungslösung nach Anspruch 1, wobei die Laugenzusammensetzung ungefähr 0,49 bis 1,45 Gew.-% NaF umfasst.

4. Reinigungslösung nach Anspruch 1 mit einer Zusammensetzung, die ungefähr 0,985 bis 8,97 Gew.-% NaOH, ungefähr 0,49 bis 1,45 Gew.-% NaF und ungefähr 89,7 bis 98,5 Gew.-% H₂O umfasst.

5. Reinigungslösung nach einem der vorhergehenden Ansprüche, die ferner ungefähr 0,15 bis 1,42 Gew.-% Na₂O(SiO₂)ₓ(H₂O)ₓ enthält.

6. Reinigungslösung nach Anspruch 5, wobei die Reinigungslösung ungefähr 0,15 bis 1,42 Gew.-% Na₂O(SiO₂)ₓ(H₂O)ₓ, ungefähr 1,90 bis 1,93 Gew.-% NaOH, ungefähr 1,43 bis 1,45 Gew.-% NaF und ungefähr 95,24 bis 96,47 Gew.-% H₂O umfasst.

7. Reinigungslösung nach einem der Ansprüche 1 bis 4, die ferner ungefähr 0,193 bis 3,54 Gew.-% Ascorbinsäure enthält.

8. Reinigungslösung nach Anspruch 7, wobei die Reinigungslösung ungefähr 0,193 bis 3,54 Gew.-% Ascorbinsäure, ungefähr 1,87 bis 1,93 Gew.-% NaOH, ungefähr 1,40 bis 1,45 Gew.-% NaF und ungefähr 93,28 bis 96,43 Gew.-% H₂O umfasst.

9. Reinigungslösung nach einem der Ansprüche 4 bis 8, die ferner einen Inhibitor zur Verhinderung der Degradation von Aluminium in den Galvanisierungsbeschichtungen oder dem Leiter enthält.

10. Reinigungslösung nach einem der Ansprüche 4 bis 9, die ferner eine Säure enthält, durch die der pH-Wert der Reinigungslösung unter 12,5 gehalten wird.

11. Verfahren zur Reinigung eines elektrischen Leiters, bei dem man:
(a) ein Leiterreinigungssystem mit
(i) einem Behälter und
(ii) einer Bewegungseinrichtung bereitstellt;
(b) eine Reinigungslösung gemäß einem der Ansprüche 1 bis 10 zum Reinigen des elektrischen Leiters bereitstellt;
(c) die Reinigungslösung in den Behälter einträgt;
(d) einen elektrischen Leiter in die Renigungslösung in dem Behälter einbringt und
(e) die Bewegungseinrichtung einschaltet, wodurch die Reinigungslösung bewegt und ihr Vermögen zum Reinigen des elektrischen Leiters erhöht wird.

12. Verfahren nach Anspruch 11, bei dem die Reinigungslösung ungefähr 0,15 bis 1,42 Gew.-% Na₂O(SiO₂)ₓ(H₂O)ₓ, ungefähr 1,90 bis 1,93 Gew.-% NaOH, ungefähr 1,43 bis 1,45 Gew.-% NaF und ungefähr 95,24 bis 96,47 Gew.-% H₂O umfasst.

13. Verfahren nach Anspruch 11, bei dem die Reinigungslösung ungefähr 0,193 bis 3,54 Gew.-% Ascorbinsäure, ungefähr 1,87 bis 1,93 Gew.-% NaOH, ungefähr 1,40 bis 1,45 Gew.-% NaF und ungefähr 93,28 bis 96,43 Gew.-% H₂O umfasst.

14. Verfahren zum Bestimmen, wann eine Reinigungslösung gemäß einem der Ansprüche 1 bis 10 in einem Leiterreinigungssystem durch eine neue Reinigungslösung zu ersetzen ist, bei dem man
(a) vor und nach jeder Reinigung von mehreren elektrischen Leitern den pH-Wert der Reinigungslösung misst;
(b) unter Verwendung der vor und nach jeder Reinigung der elektrischen Leiter vorgenommenen pH-Messungen einen pH-Abfall der Reinigungslösung für jede Reinigung berechnet;
(c) unter Verwendung der berechneten pH-Abfälle für jede Reinigung einen pH-Abfallbereich berechnet und
(d) die Reinigungslösung durch die neue Reinigungslösung ersetzt, wenn ein berechneter pH-Abfall den bestimmten pH-Abfallbereich überschreitet.

15. Verwendung einer Reinigungslösung gemäß einem der Ansprüche 1 bis 10 zum Reinigen von elektrischen Leitern.

## Revendications

1. Solution de nettoyage adaptée pour nettoyer des conducteurs électriques, comprenant : une composition caustique contenant un agent de nettoyage à base d'hydroxyde, la composition caustique contenant également du NaF.

2. Solution de nettoyage selon la revendication 1, dans laquelle la composition caustique, en pourcentage pondéral approximatif, comprend 0,985 à 8,97 % de NaOH.

3. Solution de nettoyage selon la revendication 1, dans laquelle la composition caustique, en pourcentage pondéral approximatif, comprend 0,49 à 1,45 % de NaF.

4. Solution de nettoyage selon la revendication 1, ayant une composition comprenant, en pourcentage pondéral approximatif, 0,985 à 8,97 % de NaOH, 0,49 à 1,45 % de NaF, et 89,7 à 98,5 % de H₂O.

5. Solution de nettoyage selon l'une quelconque des revendications précédentes, contenant en outre, en pourcentage pondéral approximatif, 0,15 à 1,42 % de Na₂O(SiO₂)ₓ(H₂O)ₓ.

6. Solution de nettoyage selon la revendication 5, la solution de nettoyage comprenant, en pourcentage pondéral approximatif, 0,15 à 1,42 % de Na₂O(SiO₂)ₓ(H₂O)ₓ, 1,90 à 1,93 % de NaOH, 1,43 à 1,45 % de NaF, et 95,24 à 96,47 % de H₂O.

7. Solution de nettoyage selon l'une quelconque des revendications 1 à 4, contenant en outre, en pourcentage pondéral approximatif, 0,193 à 3,54 % d'acide ascorbique.

8. Solution de nettoyage selon la revendication 7, la solution de nettoyage comprenant, en pourcentage pondéral approximatif, 0,193 à 3,54 % d'acide ascorbique, 1,87 à 1,93 % de NaOH, 1,40 à 1,45 % de NaF, et 93,28 à 96,43 % de H₂O.

9. Solution de nettoyage selon l'une quelconque des revendications 4 à 8, contenant en outre un inhibiteur pour empêcher la dégradation de l'aluminium dans les revêtements par galvanisation ou le conducteur.

10. Solution de nettoyage selon l'une quelconque des revendications 4 à 9, contenant en outre un acide pour contrôler le pH de la solution de nettoyage, de telle sorte que le pH est maintenu en dessous de 12,5.

11. Procédé de nettoyage d'un conducteur électrique, comprenant :
(a) l'obtention d'un système de nettoyage de conducteur comprenant :
(i) un récipient ; et
(ii) un agitateur ;
(b) l'obtention d'une solution de nettoyage selon l'une quelconque des revendications 1 à 10 pour nettoyer le conducteur électrique ;
(c) l'introduction de la solution de nettoyage dans le récipient ;
(d) le positionnement d'un conducteur électrique dans la solution de nettoyage disposée dans le récipient ; et
(e) l'activation de l'agitateur, pour agiter ainsi la solution de nettoyage et accroître sa capacité à nettoyer le conducteur électrique.

12. Procédé selon la revendication 11, dans lequel la solution de nettoyage comprend, en pourcentage pondéral approximatif, 0,15 à 1,42 % de Na₂O(SiO₂)ₓ(H₂O)ₓ, 1,90 à 1,93 % de NaOH, 1,43 à 1,45 % de NaF, et 95,24 à 96,47 % de H₂O.

13. Procédé selon la revendication 11, dans lequel la solution de nettoyage comprend, en pourcentage pondéral approximatif, 0,193 à 3,54 % d'acide ascorbique, 1,87 à 1,93 % de NaOH, 1,40 à 1,45 % de NaF, et 93,28 à 96,43 % de H₂O.

14. Procédé pour déterminer à quel moment remplacer une solution de nettoyage selon l'une quelconque des revendications 1 à 10 dans un système de nettoyage de conducteur par une nouvelle solution de nettoyage, comprenant :
(a) la mesure du pH de la solution de nettoyage avant et après chaque nettoyage de multiples conducteurs électriques ;
(b) le calcul de la chute de pH de la solution de nettoyage pour chaque nettoyage en utilisant les mesures de pH prises avant et après chaque nettoyage des conducteurs électriques ;
(c) la détermination d'une plage de chute de pH en utilisant les chutes de pH calculées pour chaque nettoyage ; et
(d) le remplacement de la solution de nettoyage par la nouvelle solution de nettoyage quand la chute de pH calculée dépasse la plage de chute de pH déterminée.

15. Utilisation d'une solution de nettoyage selon l'une quelconque des revendications 1 à 10 pour nettoyer des conducteurs électriques.
